



US005773706A

# United States Patent [19]

Wesley et al.

[11] Patent Number: **5,773,706**  
 [45] Date of Patent: **\*Jun. 30, 1998**

[54] **GELLED ORGANIC LIQUIDS**

[75] Inventors: **John N. Wesley, Edison; Amjad Farooq, Somerset; Ammanuel Mehreteab, Piscataway; Francis T. Barbato, Mildford, all of N.J.**

[73] Assignee: **Candle Corporation of America, Greenwich, Conn.**

[\*] Notice: The portion of the term of this patent subsequent to Oct. 15, 2014, has been disclaimed.

[21] Appl. No.: **788,487**

[22] Filed: **Jan. 28, 1997**

**Related U.S. Application Data**

[63] Continuation of Ser. No. 293,360, Aug. 19, 1994, abandoned, which is a continuation-in-part of Ser. No. 916,457, Jul. 20, 1992, abandoned.

[51] **Int. Cl.** <sup>6</sup> **B01J 13/00; C10L 7/02; C10L 7/04**

[52] **U.S. Cl.** **44/266; 44/271; 252/315.4; 252/315.7; 510/403; 510/476**

[58] **Field of Search** **252/315.4, 315.5, 252/315.6, 315.7, 314; 44/266, 271, 272; 510/403, 434**

[56] **References Cited****U.S. PATENT DOCUMENTS**

|           |         |                  |        |
|-----------|---------|------------------|--------|
| 1,523,580 | 1/1925  | Calvert          | 44/272 |
| 2,443,378 | 6/1948  | Dittmar          | 44/271 |
| 2,769,697 | 11/1956 | Goldenson et al. | 44/272 |
| 3,148,958 | 9/1964  | Monick           | 44/271 |

|           |         |               |              |
|-----------|---------|---------------|--------------|
| 3,964,880 | 6/1976  | Siegrist      | 44/266 X     |
| 4,084,939 | 4/1978  | Zmoda         | 44/271       |
| 4,205,103 | 5/1980  | Davis et al.  | 427/373      |
| 4,365,971 | 12/1982 | Monick        | 44/266       |
| 4,816,182 | 3/1989  | Novich et al. | 252/313.1    |
| 4,836,948 | 6/1989  | Corring       | 510/370      |
| 4,889,653 | 12/1989 | Ahmed et al.  | 510/223      |
| 4,904,411 | 2/1990  | Novich et al. | 252/309      |
| 4,911,857 | 3/1990  | Machin et al. | 510/369      |
| 4,956,170 | 9/1990  | Lee           | 252/315.4 X  |
| 5,053,158 | 10/1991 | Dixit et al.  | 252/174.24 X |
| 5,641,890 | 6/1997  | Wesley et al. | 44/266       |

**FOREIGN PATENT DOCUMENTS**

|         |         |                |   |
|---------|---------|----------------|---|
| 2278755 | 2/1976  | France         | . |
| 1251002 | 10/1971 | United Kingdom | . |
| 2009782 | 6/1979  | United Kingdom | . |

**OTHER PUBLICATIONS**

B.F. Goodrich, Personal Care Products Brochure, "Carbopol® Resins", pp. 1-27 (1968).  
 B F Goodrich "personal Care Products" Carbopol® Resins (1968) pp. 1-27.

*Primary Examiner*—Richard D. Lovering

[57] **ABSTRACT**

Organic liquids can be very effectively gelled by using in combination with an amine neutralized anionic polymer an auxiliary rheological additive. The auxiliary rheological additive is a substance which increases the linearity of the anionic polymer and its thixotropic properties. Suitable auxiliary rheological additives are amphoteric oxides and/or fatty acids and/or fatty acid salts. The organic liquids that can be effectively gelled are organic solvents which include fuels such as hydrocarbons and alcohols.

**19 Claims, No Drawings**

## GELLED ORGANIC LIQUIDS

This is a Continuation of application, Ser. No. 08/293, 360 filed on Aug. 19, 1994, now abandoned, which is a Continuation-in-Part of U.S. Ser. No. 07/916,457 filed Jul. 20, 1992, now abandoned.

## BACKGROUND OF THE INVENTION

This invention relates to gelled organic liquids where the structure of the organic liquids have been changed from free flowing liquids to liquids that do not flow and are considered solids under ASTM D4359-84. More particularly, this invention relates to organic liquids that can be used as fuels that are gelled to the extent that they are considered to be solids under ASTM D4359-84.

There is a need in many products to substantially increase the viscosity of organic liquids and these organic liquids may be in a mixture with water. It is easier to apply an organic liquid to a surface in a thickened condition rather than as a free flowing liquid. This is particularly the case with vertical surfaces. Products that are usefully thickened include organic based paints, paint and corrosion removers, nail polish removers, lotions, creams, salves, shampoos, household and commercial cleaners, oil drilling fluids, fuels and charcoal lighter fluids. There are yet many other uses for thickened organic liquids. When the organic liquid is gelled, it will also have a significantly reduced rate of evaporation. Due to a substantially decreased rate of evaporation the effectiveness of the organic liquid is increased.

A particularly useful area for gelled organic liquids is in gelled fuels. These can be fuels for stationary or mobile use. Gelled fuels in transport vehicles reduce the risk of fire in an accident. These gelled fuels can be used for autos, trucks, buses, boats and aircraft. This can be gelled gasoline or diesel fuel. In addition, the gelled fuels can be used as stationary sources of heat such as for cooking. A fuel of choice for such a use is an alcohol, usually methanol or ethanol, but can also be a propanol, butanol, pentanol or hexanol. Both methanol and ethanol are commonly used fuels for cooking. The gelled methanol or ethanol in one use is in a container that has a capacity of about 200 to 500 ml. This container is placed under a chafing dish and ignited to keep the food contents of the chafing dish warm. These containers will burn from about 2 to 5 hours depending on the volume of the fuel in the container.

Fuels to be effectively used without a wick to deliver the fuel to a burn surface must be gelled. Further, these fuels should be gelled so that they are classified as solids under ASTM D4359-84. The fuel must not separate from the gel on standing or upon the application of pressure. The primary reason is safety. If a gelled fuel is classified as a solid under ASTM D4359-84 it will be subject to less vigorous regulations for transport and storage.

A commonly used gelling agent for commercially available fuels such as methanol or ethanol is nitrocellulose. The nitrocellulose holds the fuel in a sponge-like matrix. However, this is not a true gel. Some of the fuel can be physically separated from the nitrocellulose. The net result is that in a container there can be free fuel present. This is not desirable.

In U.S. Pat. No. 3,759,674 there is disclosed dispersions of certain ethylene-acrylic acid copolymers and amine emulsifiers in water to be admixed with alcohols. The dispersions contain from 10 to 20 parts by weight of the ethylene-acrylic acid copolymer and from about 3 to 4 parts by weight of an amine emulsifier. It will be from about 10 to 30 percent by

weight solids. In U.S. Pat. No. 3,148,958 there is disclosed the gelling of an alcohol fuel through the use of carboxy vinyl polymers neutralized with a weak amine base. This results in a gelled alcohol fuel that is stated to have good burn characteristics. U.S. Pat. No. 4,261,700 and U.S. Pat. No. 4,365,971 each disclose the use of a Carbopol 934 ethylene acrylic acid copolymer gelling agent for an alcohol fuel. The Carbopol 934 is neutralized to form the gel using a weak amine base. In U.S. Pat. No. 3,214,252 there is disclosed the use of olefin-maleic anhydride copolymers as gelling agents for alcohols. These are gelled by compounds that can supply an hydroxyl group. In U.S. Pat. No. 4,536,188 there is disclosed the incorporation of alcohol-soluble metal compounds into an alcohol fuel to increase the visibility of the otherwise invisible flames. It is also known from U.S. Pat. No. 2,890,257 to add silica gel or activated aluminas to stabilize naptha fuels. These are not gelled fuels. It is also known to gel a range of solvents using amine neutralized polyacrylic acid polymers.

The disclosures of these references are interesting but there is no directions to gel a solvent by the use of an alkaline compound such as an amine neutralized anionic polymer which contains an auxiliary rheological additive to increase the linearity of the anionic polymer. An auxiliary Theological additive is a substance that increases the viscosity of a solution of the amine neutralized anionic polymer. Upon the anionic polymer being dissolved and neutralized there is an increase in anionic polymer linearity. This linearity is further enhanced through the use of an auxiliary rheological additive. It has also been found that when the solvent is a fuel, such as an alcohol fuel, that the use of an agent for the structuring of the polymer, such as an amphoteric metal oxide, and optionally a fatty acid, a fatty alcohol or a salt of a fatty acid, provides for a more effective burning of the fuel as well as a more cost effective fuel source. It appears that a solid amphoteric metal oxide decreases the tendency of the burn surface to form a continuous skin seal. When such a skin seal is formed, the fuel has to erupt through the skin to burn. This produces noise and irregular burning. This does not occur when an amphoteric oxide auxiliary Theological additive is used. There is also an improved gel. In addition, the replacement part of the anionic polymer content with the lower cost auxiliary rheology additive results in lower cost products.

## BRIEF SUMMARY OF THE INVENTION

The present invention is directed to producing improved gelled solvents, and in particular, organic solvents. The gelled organic solvents include alkanes, alkenes, aromatics, acids, ketones, aldehydes, oils, ethylene glycols, polyethylene glycols, amines, alcohols and esters. The gelled solvents have a wide area of usage. One particular area of usage is as gelled fuels, and in one preferred embodiment as gelled fuels for cooking and heating foods.

The gelled solvents will contain from about 0.1 to 10 weight percent of a base neutralized anionic polymer, 0.01 to 10 weight percent of an auxiliary rheological additive with the balance being at least one solvent, and primarily an organic solvent. Water can be present as a part of the solvent. The neutralized anionic polymer is preferably an amine neutralized cross-linked anionic polymer such as a cross-linked polyacrylic acid polymer and has a molecular weight of about 60,000 to 10,000,000. The polyacrylic acid polymer is neutralized using an amine base. The presence of an auxiliary Theological additive, which serves to further uncoil the anionic polymer and thus increase its linearity, increases the thixotropic properties of the gelled organic

solvent. There is an increase in viscosity of from about 10 to 300 percent of the viscosity of a similar gelled solvent which does not contain the auxiliary Theological additive.

#### DETAILED DESCRIPTION OF THE INVENTION

This invention is directed to gelled solvents, and in particular to gelled organic solvents. The gelled organic solvents can contain some water, but since the organic is predominant it will be considered to be a gelled organic solvent. The water content can range from about 0 to about 45 wt. percent, and in many cases 0.1 to 35 wt. percent of the gelled composition. In a particular embodiment the invention is directed to gelled fuels. The organic fuel component can be an alkane, alkene, alcohol, ester, an aromatic or mixtures of these hydrocarbons. In a preferred embodiment the fuel is an alcohol of from 1 to 6 carbon atoms.

The combination of the base neutralized, and usually amine neutralized, crosslinked anionic polymeric and the auxiliary rheological additive results in enhanced thixotropic properties. The auxiliary rheological additive will increase the viscosity of the gelled solvent from about 10 to 300 percent. This is a significant increase for the addition of a relatively small amount of an additive.

The polymer thickening agents and auxiliary rheological additives both contribute to the viscoelastic rheology of the thickened compositions of the instant invention. As used herein, "viscoelastic" or "viscoelasticity" means that the elastic (storage) moduli ( $G'$ ) and the viscous (loss) moduli ( $G''$ ) are both substantially independent of strain, at least in an applied torque range of from 1 to 150 micro N.m (Newton meter). More specifically, a composition is considered to be linear viscoelastic for purposes of this invention, if over the torque range of 1 to 150 micro N.m the elastic moduli  $G'$  has a minimum value of at least 2,500 dynes/sq. cm., preferably at least 3,500 dynes/sq.cm., and varies less than 500 dynes/sq. cm, preferably less than 400 dynes/sq. cm., and especially preferably less than 370 dynes/sq.cm. Typically, the variation in viscous (loss) moduli  $G''$  will be less than that of  $G'$ . As a further characteristic of the preferred linear viscoelastic compositions the ratio of  $G''/G'$  ( $\tan\delta$ ) is less than 1, preferably less than 0.4, and more preferably less than 0.2, at least over the torque range of 1 to 150 micro N.m.

By way of further explanation, the elastic (storage) modulus  $G'$  is a measure of the energy stored and retrieved when a strain is applied to the composition while viscous (loss) modulus  $G''$  is a measure to the amount of energy dissipated as heat when strain is applied. Therefore, a value of  $\tan\delta$ ,

$$0.05 < \tan\delta < 1,$$

preferably

$$0.2 > \tan\delta < 0.8$$

means that the compositions will retain sufficient energy when a stress or strain is applied. The compositions with  $\tan\delta$  values in these ranges, therefore, will also have a high cohesive property, namely, when a shear or strain is applied to a portion of the composition to cause it to flow, the surrounding portions will follow. As a result of this cohesiveness of the subject viscoelastic compositions, the compositions will readily flow uniformly and homogeneously thereby contributing to the physical (phase) stability of the formulation which characterizes the present compositions. The viscoelastic property also contributes to improved

physical stability against phase separation of any undissolved suspended particles by providing a resistance to movement of the particles due to the strain exerted by a particle on the surround fluid medium.

5 A means for further improving the structuring of the gel formulations in order to obtain improved viscosity as well as  $G'$  and  $G''$  values is to form a solution of an organic solvent, a neutralized cross-linked anionic polymer such as a neutralized cross-linked polyacrylic acid thickening agent by 10 mixing at room temperature to slightly elevated temperature and subsequently with mixing neutralizing the anionic groups, such as the carboxylic acid groups, by the addition of an excess basic material, such as an organic amine, to form a neutralized cross-linked anionic polymer such as a 15 cross-linked polyacrylic acid polymer having a molecular weight of about 60,000 to 10,000,000. To the solution of the amine neutralized cross-linked anionic polymer is added with mixing an auxiliary rheological additive such as an amphoteric metal oxide which is a colloidal, insoluble 20 particulate such as aluminum oxide and/or a fatty acid and/or a salt of a fatty acid and/or a fatty alcohol. The neutralized crosslinked anionic polymer such as a cross-linked polyacrylic acid polymer in combination with the auxiliary rheological additive provides improved  $G'$  and  $G''$  25 values as well as improved viscosification of the organic polymeric solution which has a pH of about 7 to 14 as compared to the use of the neutralized cross-linked anionic polymer alone. It is theorized that the improvement in viscosification results from an increase in solid content and 30 from the association of the amphoteric metal oxide and the neutralized cross-linked anionic polymer in the organic solvent, wherein an uncoiling of the polymeric chain of the neutralized and cross-linked anionic polymer, such as a polyacrylic acid, occurs which provides a further building of 35 the polymeric structure within the organic solvent. To the solution of the neutralized cross-linked polyacrylic acid polymer, solvent and auxiliary rheological additive can be added various other ingredients to form fuel compositions, an after shave gel, a detergent composition, a hard surface 40 cleaning composition or any of the previously mentioned compositions. Other commercial and industrial compositions can be formed for a variety of applications such as fabric cleaners, shampoos, floor cleaners, cleaning paste, tile cleaners, ointments, oven cleaners, pharmaceutical 45 suspensions, concentrated coal slurries, oil drilling muds, cleaning prespotters and organic solvent based paints. These compositions can be formulated by adding the appropriate chemicals to the polymeric solution of neutralized cross-linked polyacrylic acid polymer, organic solvent, and the 50 auxiliary rheological additive to form the desired composition. The organic solution of organic solvent, neutralized cross-linked anionic polymer such as a polyacrylic acid polymer and the auxiliary Theological additive such as an amphoteric metal oxide has a complex viscosity at room 55 temperature at 10 radians/second of 1 to 1,000 dyne seconds/sq. cm., more preferably 30 to 800 dyne seconds/sq. cm.. The organic solution comprises 0.01 to 10 weight %, more preferably 0.02 to 5 weight % of a auxiliary Theological additive, 0.1 to 10 weight %, and more preferably 0.1 to 5 weight % of a base neutralized, cross-linked anionic polymer such as an amine neutralized, cross-linked polyacrylic polymer, and the balance being an organic solvent, mixtures of organic solvents, or mixtures of organic solvents and water wherein the polymeric solution has a  $G'$  value of at 60 least 2,500 dynes/sq. cm at a frequency of 10 radians/second, a  $G''$  value of at least 200 dynes/sq. cm. at a frequency of 10 radians/second, a ratio of  $G''/G'$  is less than 65

1 and G' is substantially constant over a torque range of 1 to 150 micro N.m.

If the organic solution has a G' value of a least 80 dynes/sq. cm. at a frequency of 10 radians/second and the G" value is at least 10 dynes/sq. cm. at a frequency of 10 radians/second, wherein G' is substantially constant over a torque range of 1 to 100 micro N.m and a ratio of G"/G' is less than 1 and a yield stress of at least 5 dynes/sq. cm. more preferably 1 to 1200 dynes/sq. cm., the organic solution will be a gel which can function as a suspension medium for a plurality of solid particles, immiscible liquid droplets or gaseous bubbles. The solid particles, liquid droplets or gaseous bubbles can be inorganic, organic or polymeric. The solid material, liquid droplets or gaseous bubbles which are not soluble in the solvent, should not decompose in the solvent or react with the anionic groups of the anionic polymer. The concentration of the solid particles, liquid droplets or gaseous bubbles in the suspension medium is 0.1 to 70 weight percent, more preferably 1 to 50 weight %.

The estimated minimum yield stress of the gel suspension medium which is necessary to suspend each of the solid spherical particles, liquid droplets or gaseous bubbles such that the particles, droplets or bubbles remain suspended for at least seven days in the gel suspension medium is expressed by the equation:

$$\text{minimum yield stress} = \frac{4(\Delta P)gR^3}{3A}$$

wherein R equals the radius of each of the solid particles, liquid droplets and/or gaseous bubbles; g equals the gravitational constant;  $\Delta P$  equals the difference between the density of the gel suspension medium and the density of each of the solid particles, liquid droplets or gaseous bubbles and A equals the surface area of each of the solid particles, liquid droplets or the gaseous bubbles.

Additionally, by way of explanation, it is necessary to clearly emphasize that in order to minimize the rate and amount of sedimentation of solid particles that are insoluble in the suspension medium that the suspension medium should exhibit strain independent moduli. For materials that exhibit strain independence of the viscoelastic moduli (G'), these materials tend to exhibit a critical property known as the yield stress which prevents the sedimentation of insoluble particles from the suspension medium. It is also critical in the understanding of the data as presented in this invention that by linear viscoelastic gel it is meant that G' is substantially constant over a torque range of 1 to 150 micro N.m. The minimum estimated yield stress for the gel necessary to suspend each of the spherical particles in the gel such that each particle will not precipitate from the gel is expressed by the formula:

$$\text{minimum yield stress} = \frac{4(\Delta P)gR^3}{3A} \text{ dynes/sq. cm}$$

wherein R equals the radius of each of the solid particle, A equals the surface area of each of the solid particle, g equals the gravitational constant and  $\Delta P$  equals the difference in density between the gel and the density of each of the solid particles.

Illustrative of amine neutralized anionic polymers contemplated within the scope of the instant invention beside the polyacrylic acid polymers such as the Carbopols are: sulfonated polymers containing a sulfonate functionality as defined in U.S. Pat. Nos. 3,642,728; 4,608,425; 4,619,773; 4,626,285; 4,637,882; 4,640,945; 4,647,603; 4,710,555; 5,730,028; 4,963,032; 4,963,032; 4,970,260 and 4,975,82,

wherein these patents are all hereby incorporated by reference, as well as polymers and monomers containing a carboxylic acid functionally as defined in U.S. Pat. Nos. 4,612,332; 4,673,716; 4,694,046; 4,694,058; 4,709,759; 4,734,205; 4,780,517; 4,960,821 and 5,036,136, wherein these patents are all hereby incorporated by reference, as well as copolymers containing a maleic anhydride functionality such as a cross-linked Gantrez provided that there is a sufficient association between the amine neutralized salts of these polymers in the aforementioned patents and the auxiliary Theological additive to create a viscoelastic gel having the G' and G" properties as defined herein.

Exemplary of the cross-linked polyacrylic acid-type thickening agents are the products sold by B.F. Goodrich under their Carbopol trademark, especially Carbopol 941, which is the most ion-insensitive of this class of polymers, and Carbopol 676, Carbopol 940 and Carbopol 934. The Carbopol resins, also known as "Carbomer", are hydrophilic high molecular weight, cross-linked acrylic acid polymers having an average equivalent weight of 76, and the general structure illustrated by the following formula:



Carbopol 941 has a molecular weight of 1,250,000; Carbopol 940 a molecular weight of approximately 4,000,000 and Carbopol 934 a molecular weight of approximately 3,000,000. The Carbopol resins are cross-linked with poly-alkenyl polyether, e.g. 1% of a polyallyl ether of sucrose having an average of 5.8 allyl groups for each molecule of sucrose. Further detailed information on the Carbopol resins is available from B.F. Goodrich, see, for example, the B.F. Goodrich catalog GC-67, Carbopol® Water Soluble Resins.

While favorable results have been achieved with Carbopol 941 polyacrylic resin, other lightly cross-linked polyacrylic acid-type thickening agents can also be used in the compositions of this invention. As used herein "polyacrylic acid-type" refers to homopolymers of acrylic acid or methacrylic acid or copolymers of these acids or their salts, esters or amides with each other or with one or more other ethylenically unsaturated monomers, such as, for example styrene, maleic acid, maleic anhydride, 2-hydroxyethylacrylate, acrylonitrile, vinyl acetate, ethylene, propylene, and the like.

The Carbopol 600 series resin are the most useful in the instant invention. These are salt insensitive, high molecular weight polyacrylic acids which are cross-linked with poly-alkenyl ether. In addition to the or branched nature of these resins, they are more highly cross-linked than the 900 series resins and have molecular weights between about 1,000,000 and 4,000,000. Very useful of the Carbopol 600 series resins is Carbopol 614. Carbopol 614 is also highly stable to any anticipated storage temperature conditions from below freezing to elevated temperatures as high as 120° F., preferably 140° F., and especially 160° F., for periods of as long as several days to several weeks or months or longer.

The homopolymers or copolymers are characterized by their high molecular weight, in the range of from 60,000 to 10,000,000, preferably 500,000 to 5,000,000, especially from 1,000,000 to 4,000,000, and by their organic solvent solubility. These thickening agents are used in their lightly cross-linked form wherein the cross-linking may be accomplished by means known in the polymer arts, as by

irradiation, or, preferably, by the incorporation into the monomer mixture to be polymerized of known chemical cross-linking monomeric agents, typically polyunsaturated (e.g. diethylenically unsaturated) monomers, such as, for example, divinylbenzene, divinylether of diethylene glycol, N, N'-methylene- bisacrylamide, polyalkenylpolyethers (such as described above, and the like. Typically, amounts of cross-linking agent to be incorporated in the final polymer may range from 0.01 to 1.5 percent, preferably from 0.05 to 1.2 percent, and especially, preferably from 0.1 to 0.9 percent, by weight of cross-linking agent to weight of total polymer. Generally, those skilled in the art will recognize that the degree of cross-linking should be sufficient to impart some coiling of the otherwise generally linear polymeric compound. It is also understood that the water-swelling of the polymer which provides the desired thickening and viscous properties generally depends on one or two mechanisms, namely, conversion of the acid group containing polymers to the corresponding salts, e.g. sodium, generating negative charges along the polymer backbone, thereby causing the coiled molecules to expand and thicken the aqueous solution; or by formation of hydrogen bonds, for example, between the carboxyl groups of the polymer and a hydroxyl donor. The latter mechanism is especially important in the present invention, and therefore, the preferred polyacrylic acid-type thickening agents will contain free carboxylic acid (COOH) groups along the polymer backbone. Also, it will be understood that the degree of cross-linking should not be so high as to render the cross-linked polymer completely insoluble or non-dispersible in water and/or organic solvents or inhibit or prevent the further uncoiling of the polymer molecules in the presence of the amphoteric metal oxide.

The amount of the cross-linked anionic polymer such as a high molecular weight, cross-linked polyacrylic acid or other high molecular weight, hydrophilic crosslinked polyacrylic acid-type thickening agent to impart the desired Theological property of linear viscoelasticity will generally be in the range of from 0.1 to 10%, preferably from 0.1 to 5% and most preferably about 0.2 to 1% by weight, based on the weight of the composition, although the amount will depend on the particular cross-linking agent, ionic strength of the composition, hydroxyl donors and the like.

The auxiliary rheological additive can be a colloidal thickener which preferably is an amphoteric metal oxide

which has an average particle size diameter in dispersion of about 0.05 to 2.0 microns, more preferably about 0.05 to about 1.1 microns. Because of their particle size of less than 1 micron these amphoteric metal oxides are non abrasive. The dispersion of the metal oxide contains about 60 to about 90 wt. percent of the metal oxide and the dispersion has a pH of about 3 to about 4. When the acid dispersion of the metal oxide is added to the basic solution of the neutralized anionic polymer, the acidic dispersion of the metal oxide is neutralized thereby making the dispersion of the metal oxide effective as an auxiliary Theological additive. A preferred metal oxide is aluminum oxide. Useful aluminum oxide dispersions are sold by Vista Chemical Company of Houston, Texas under the tradename Dispal Alumina 23 N4-80, Dispal Alumina 23 N4-20 or Dispal Alumina T23. The auxiliary rheological additive may also be a fatty acid or a salt of a fatty acid or a fatty alcohol. In addition, a fatty acid, fatty alcohol or a salt of a fatty acid in combination with the amphoteric oxide may function as the auxiliary rheological additive.

The anionic cross-linked polymer can be neutralized with an organic amine. The organic amine that can be used to neutralized the anionic polymer can be a primary, secondary or tertiary aliphatic amine, aromatic amine or a heterocyclic amine, wherein the aliphatic amines are especially preferred. For example, in the case of an amine neutralized cross-linked Carbopol polymer, some amines which can be used to neutralize the cross-linked Carbopol polymer are diisopropanolamine, Ethomeen C25, Di-2 ethylhexyl amine, triethanol amine, triamyl amine, dimethylaminopropionitrile, alamine, dodecylamine, a copolymer of ethylene/vinyl pyridene and morpholine. Mixed systems of an alkali metal neutralized cross-linked anionic polymer and an amine neutralized cross-linked anionic polymer can at times be employed, wherein the ratio of the metal neutralized polymer to the amine neutralized polymer can be 100/1 to 1/100 and more preferably 10/1 to 1/10. The selection of the neutralizing agent for the anionic polymer is governed, in part by the solvent system of the composition. Typical solvents that can be employed to dissolve the amine neutralized cross-linked anionic polymers and which are consequently gelled are illustrated in Table I. The gelling is with the use of the above enumerated amines.

TABLE I

| % Solvent A<br>% Solvent B | (1) | (2) | (3) | (4) | (5) | (6) | (7) | (8) | (9) | (10) | (11) |
|----------------------------|-----|-----|-----|-----|-----|-----|-----|-----|-----|------|------|
| 90 Ethanol                 |     |     |     | X   |     |     |     |     |     |      |      |
| 10 DMF                     |     |     |     |     |     |     |     |     |     |      |      |
| 90 Ethanol                 | X   | X   | X   |     |     |     |     |     |     |      |      |
| 10 Methanol                |     |     |     |     |     |     |     |     |     |      |      |
| 90 Ethanol                 | X   | X   | X   |     |     | X   |     |     |     |      |      |
| 10 Water                   |     |     |     |     |     |     |     |     |     |      |      |
| Ethyl formamide            | X   | X   | X   |     |     |     |     |     |     |      |      |
| Ethylene glycol            | X   | X   |     |     |     |     |     |     |     |      | X    |
| 90 Ethylene glycol         | X   | X   |     |     |     |     |     |     |     |      |      |
| 10 DMF                     |     |     |     |     |     |     |     |     |     |      |      |
| 90 Ethylene glycol         | X   | X   |     |     |     |     |     |     |     |      | X    |
| 10 Methanol                |     |     |     |     |     |     |     |     |     |      |      |
| 90 Ethylene glycol         | X   | X   |     |     |     |     |     |     |     |      | X    |
| 10 Water                   |     |     |     |     |     |     |     |     |     |      |      |
| Ethylene oxide             |     |     | X   | X   |     |     |     |     | X   |      |      |
| Glycerol                   | X   |     |     |     |     |     |     |     |     |      | X    |
| 80 Hexane                  |     |     |     |     |     |     |     |     |     | X    |      |
| 20 Methanol                |     |     |     |     |     |     |     |     |     |      |      |
| 90 Isopropanol             |     |     |     | X   |     |     |     |     |     |      |      |

TABLE I-continued

| % Solvent A<br>% Solvent B | (1) | (2) | (3) | (4) | (5) | (6) | (7) | (8) | (9) | (10) | (11) |
|----------------------------|-----|-----|-----|-----|-----|-----|-----|-----|-----|------|------|
| 10 Water                   |     |     |     |     |     |     |     |     |     | X    | X    |
| 90 Metaxylene              |     |     |     |     |     |     |     |     |     |      |      |
| 10 Methanol                |     |     |     |     |     |     |     |     |     |      |      |
| Methanol                   | X   | X   | X   |     | X   |     |     | X   |     |      |      |
| 90 Methanol                | X   | X   | X   |     |     |     |     |     |     | X    |      |
| 10 DMF                     |     |     |     |     |     |     |     |     |     |      |      |
| Methyl                     | X   | X   | X   |     |     |     |     |     |     |      |      |
| Cellosolve                 |     |     |     |     |     |     |     |     |     |      |      |
| n-methyl-2-pyrrolidone     |     |     | X   |     |     |     |     |     |     |      |      |
| 90 Mineral spirits         |     |     |     |     |     |     | X   |     | X   |      |      |
| 10 Methanol                |     |     |     |     |     |     |     |     |     |      |      |
| Nitrobenzene               |     | X   |     |     |     |     |     |     |     |      |      |
| 90 Nitrobenzene            |     | X   |     |     |     |     |     |     |     |      |      |
| 10 DMF                     |     |     |     |     |     |     |     |     |     |      |      |
| 90 Nitrobenzene            |     | X   |     |     |     |     |     |     |     |      |      |
| 10 Methanol                |     |     |     |     |     |     |     |     |     |      |      |
| Phenyl acetate             |     |     | X   |     |     |     |     |     |     |      |      |
| 90 Diacetone alcohol       | X   | X   |     | X   |     |     |     |     |     |      |      |
| 10 Water                   |     |     |     |     |     |     |     |     |     |      |      |
| Diethyl acetamide          | X   | X   |     |     |     |     |     |     |     |      |      |
| Diethyl formamide          | X   | X   |     | X   |     |     | X   |     |     |      |      |
| 90 Diethyl formamide       | X   | X   |     | X   |     |     |     | X   |     |      |      |
| 10 DMF                     |     |     |     |     |     |     |     |     |     |      |      |
| 90 Diethyl formamide       | X   | X   |     | X   |     |     |     | X   |     |      |      |
| 10 Methanol                |     |     |     |     |     |     |     |     |     |      |      |
| Diethylene glycol          | X   | X   | X   |     |     |     |     |     |     |      |      |
| Dimethyl acetamide         |     | X   | X   |     |     |     | X   |     |     |      |      |
| 1,4 Dioxane                |     |     | X   |     |     |     |     |     |     |      |      |
| Dipropyl sulfone           | X   | X   | X   |     |     |     | X   |     | X   |      |      |
| Dimethyl formamide (DMF)   | X   | X   | X   |     |     |     | X   | X   | X   |      |      |
| 95 DMF                     |     |     | X   | X   |     |     |     |     |     |      |      |
| 5 Ethylene glycol          |     |     |     |     |     |     |     |     |     |      |      |
| 90 DMF                     | X   | X   | X   |     |     |     | X   | X   | X   |      |      |
| 10 Methanol                |     |     |     |     |     |     |     |     |     |      |      |
| 90 DMF                     |     | X   |     |     |     |     |     |     |     |      |      |
| 10 Water                   |     |     |     |     |     |     | X   |     |     |      |      |
| 60 DMF                     |     | X   | X   |     |     |     |     |     |     |      |      |
| 60 Acetone                 |     |     |     |     |     |     |     |     |     |      |      |
| 50 DMF                     |     |     | X   |     |     |     |     |     |     |      |      |
| 50 Toluene                 |     |     |     |     |     |     |     |     |     |      |      |
| Dimethyl sulfoxide (DMSO)  | X   | X   | X   | X   | X   |     | X   |     | X   |      |      |
| 90 DMSO                    | X   | X   | X   |     |     |     |     |     | X   |      |      |
| 10 DMF                     |     |     |     |     |     |     |     |     |     |      |      |
| 90 DMSO                    |     | X   | X   |     |     |     |     |     |     |      |      |
| 10 Methanol                |     |     |     |     |     |     |     |     |     |      |      |
| 90 DMSO                    |     |     | X   |     |     |     |     |     |     |      |      |
| 10 Water                   |     |     |     |     |     |     |     |     |     |      |      |
| Ethanol                    | X   | X   | X   |     |     |     | X   |     |     |      |      |
| 95 Ethanol                 | X   | X   | X   |     |     |     |     |     |     |      |      |
| 5 Ethylene glycol          |     |     |     |     |     |     |     |     |     |      |      |
| 90 Ethanol                 | X   | X   | X   |     |     |     |     |     |     |      |      |
| 10 Ethylene glycol         |     |     |     |     |     |     |     |     |     |      |      |
| 90 Acetone                 |     | X   | X   |     |     |     | X   |     |     |      |      |
| 10 Methanol                |     |     |     |     |     |     |     |     |     |      |      |
| 80 Acetone                 |     | X   | X   |     |     |     | X   |     |     |      |      |
| 20 Methanol                |     |     |     |     |     |     |     |     |     |      |      |
| 90 Acetone                 |     | X   | X   |     |     |     | X   |     |     |      |      |
| 10 Water                   |     |     |     |     |     |     |     |     |     |      |      |
| 80 Acetone                 | X   | X   | X   |     |     |     | X   |     |     |      |      |
| 20 Water                   |     |     |     |     |     |     |     |     |     |      |      |
| Acetonitrile               | X   | X   | X   |     | X   | X   |     | X   |     |      |      |
| 95 Acetonitrile            | X   | X   | X   | X   | X   |     |     | X   |     |      |      |
| 5 Ethylene glycol          |     |     |     |     |     |     |     |     |     |      |      |
| 90 Acetonitrile            |     | X   |     |     |     |     | X   |     |     |      |      |
| 10 DMF                     |     |     |     |     |     |     |     |     |     |      |      |
| 90 Acetonitrile            | X   | X   | X   |     |     |     | X   |     |     |      |      |
| 10 Methanol                |     |     |     |     |     |     |     |     |     |      |      |
| 90 Acetonitrile            | X   | X   | X   | X   | X   |     | X   | X   | X   | X    |      |
| 10 Water                   |     |     |     |     |     |     |     |     |     |      |      |
| Acetyl acetone             | X   | X   |     |     |     |     |     |     |     |      |      |
| Acrylonitrile              | X   | X   |     |     |     |     |     |     |     |      |      |
| Aniline                    | X   | X   |     |     |     |     |     |     |     |      |      |
| Benzonitrile               | X   | X   |     |     |     |     | X   |     | X   |      |      |

TABLE I-continued

| % Solvent A<br>% Solvent B | (1) | (2) | (3) | (4) | (5) | (6) | (7) | (8) | (9) | (10) | (11) |
|----------------------------|-----|-----|-----|-----|-----|-----|-----|-----|-----|------|------|
| Benzyl alcohol             | X   | X   |     |     |     |     |     |     |     |      |      |
| Butyl Carbitol             |     |     | X   |     |     |     |     |     |     |      |      |
| Butyl Cellosolve           |     |     | X   |     |     |     |     |     |     |      |      |
| Butyrol acetone            | X   |     | X   |     |     |     |     |     |     |      |      |
| Butyrolactone              | X   | X   | X   |     |     |     |     |     |     |      |      |
| 70 Carbitol                |     |     | X   |     |     |     |     |     |     |      |      |
| 30 Methanol                |     |     |     |     |     |     |     |     |     |      |      |
| 90 Carbon tetrachloride    |     | X   | X   |     |     |     |     |     |     |      | X    |
| 10 Methanol                |     |     |     |     |     |     |     |     |     |      |      |
| Diacetone alcohol          |     | X   | X   |     |     |     |     |     |     |      |      |
| 90 Diacetone alcohol       |     |     | X   |     |     |     |     |     |     |      |      |
| 10 DMF                     |     |     |     |     |     |     |     |     |     |      |      |
| 90 Diacetone alcohol       |     | X   | X   |     |     |     |     |     |     |      |      |
| 10 Ethylene glycol         |     |     |     |     |     |     |     |     |     |      |      |
| 90 Diacetone alcohol       |     | X   | X   |     |     |     |     |     |     |      |      |
| 10 Methanol                |     |     |     |     |     |     |     |     |     |      |      |
| n-propanol                 |     |     | X   |     |     |     |     |     |     |      |      |
| 90 n-propanol              |     |     | X   |     |     |     |     |     |     |      | X    |
| 10 Water                   |     |     |     |     |     |     |     |     |     |      |      |
| Propiolactone              | X   | X   | X   |     |     |     |     |     |     |      |      |
| Propionitrile              |     |     | X   | X   |     |     |     |     |     |      |      |
| Propylene glycol           | X   | X   | X   |     | X   |     |     |     |     |      |      |
| 90 Propylene glycol        | X   | X   |     |     |     |     |     |     |     |      | X    |
| 10 Methanol                |     |     |     |     |     |     |     |     |     |      |      |
| 90 Propylene glycol        |     | X   | X   |     |     |     |     |     |     |      |      |
| 10 Water                   |     |     |     |     |     |     |     |     |     |      |      |
| Styrene                    |     | X   | X   | X   |     |     |     |     |     |      | X    |
| 90 Toluene                 |     |     |     |     |     |     |     |     |     |      | X    |
| 10 Ethanol                 |     |     |     |     |     |     |     |     |     |      |      |
| 90 Toluene                 |     |     |     |     |     |     |     |     |     |      | X    |
| 10 Methanol                |     |     |     |     |     |     |     |     |     |      |      |
| Water                      |     | X   | X   |     | X   | X   | X   | X   | X   | X    |      |
| 90 Xylene                  |     |     |     |     |     |     |     |     |     |      | X    |
| 10 Methanol                |     |     |     |     |     |     |     |     |     |      |      |
| 90 Orthoxylene             |     |     |     |     |     |     |     |     |     |      | X    |
| 10 Methanol                |     |     |     |     |     |     |     |     |     |      |      |
| 90 Paraxylene              |     |     |     |     |     |     |     |     |     |      | X    |
| 10 Methanol                |     |     |     |     |     |     |     |     |     |      |      |

(1) Diisopropanolamine

(2) Ethomeen (BASF-Wyandotte Corp)

(3) Di2 (ethyl hexyl) amine

(4) Triethanolamine

(5) Triamylamine

(6) Jeffamine D-1000 (Jefferson Chemical Company Inc.)

(7) b-Dimethylaminopropionitrile

(8) Armeen (Armak Industrial Chemical Division)

(9) Alamine 7D (Henkel Corporation)

(10) Dodecylamine

(11) Morpholine

Long chain fatty alcohols, fatty acids or monovalent or polyvalent salts thereof can be used alone as an auxiliary rheological additive or in combination with the aforementioned colloidal amphoteric oxides. Although the manner by which the fatty alcohol, fatty acid or salt contributes to the rheology and stability of the composition has not been fully elucidated it is hypothesized that it may function as a hydrogen bonding agent or cross-linking agent.

The preferred long chain fatty alcohols and fatty acids are the higher aliphatic fatty alcohols and fatty acids having from 8 to 22 carbon atoms, more preferably from 10 to 20 carbon atoms, especially preferably from 12 to 18 carbon atoms, inclusive of the carbon atom of the alcohol or carboxyl group. The aliphatic radical may be saturated or unsaturated and may be straight or branched. Straight chain saturated fatty alcohols and fatty acids are preferred. Mixtures of fatty alcohols and fatty acids may be used. Examples of fatty acids are those derived from natural sources, such as tallow fatty acid, coco fatty acid, soya fatty acid, mixtures of these acids, etc. Stearic acid and mixed fatty acids, e.g. stearic acid/palmitic acid, are preferred. The fatty alcohols are derived from the reduction of the counterpart fatty acid.

When the free acid form of the fatty acid is used directly it will generally associate with any potassium and sodium ions to form the corresponding alkali metal fatty acid soap. However, the fatty acid salts may be directly added to the composition as sodium salt or potassium salt, or as a polyvalent metal salt, although the alkali metal salts of the fatty acids are preferred fatty acid salts.

The preferred polyvalent metals are the di- and tri- valent metals of Groups IIA, IIB and IIIB, such as magnesium, calcium, aluminum and zinc, although other polyvalent metals, including those of Groups IIIA, IVA, VA, IB, IVB, VB, VIB, VIIB and VIII of the Periodic Table of the Elements can also be used. Specific examples of such other polyvalent metals include Ti, Zr, V, Nb, Mn, Fe, Co, Ni, Cd, Sn, Sb, Bi, etc. Generally, the metals may be present in the divalent to pentavalent state. Preferably the metal salts are used in their higher oxidation states.

The amount of the fatty alcohol, fatty acid or fatty acid salt stabilizer and/or colloidal thickener to achieve the desired enhancement of physical stability will depend on such factors as the nature of the colloidal amphoteric oxide,

the fatty alcohol, fatty acid or its salt, the nature and amount of the polymeric thickening agent, the nature and amount of the organic solvent and other ingredients, as well as the anticipated storage and shipping conditions.

Generally, however, amounts of the fatty alcohol, fatty acid or fatty acid salt stabilizing agents in the range of from about 0.01 to 4%, preferably 0.02 to 2%, more preferably from 0.02 to 0.8%, especially preferably from 0.08 to 0.4%, provide a long term stability and absence of phase separation upon standing or during transport at both low and elevated temperatures as are required for commercially acceptable product.

A further means of improving the thickening of the polymeric solutions of the instant invention comprises using in combination with the neutralized anionic polymer an inorganic layered colloidal forming clay such as a laponite clay, a smectite clay or an attapulgite clay. The concentration of the clay in the instant composition is about 0.1 to about 10 wt. percent, more preferably about 0.2 to about 4 wt. percent.

Smectite clays include montmorillonite (bentonite), hectorite, smectite, saponite, and the like. Montmorillonite clays are preferred and are available under tradenames such as Thixogel (Registered trademark) No. 1 and Gelwhite (Registered Trademark) GP, H, etc., from Georgia Kaolin Company; and ECCAGUM (Registered Trademark) GP, H, etc., from Luthern Clay Products. Attapulgite clays include the materials commercially available under the tradename Attagel (Registered Trademark), i.e. Attagel 40, Attagel 50 and Attagel 150 from Engelhard Minerals and Chemicals Corporation. Mixtures of smectite and attapulgite types in weight ratios of 4:1 to 1:5 are also useful herein. Thickening or suspending agents of the foregoing types are well known in the art, being described, for example, in U.S. Pat. No. 3,985,668 referred to above.

The layered clay minerals suitable for use in the present invention belong to the geological classes of the smectites, the kaolins, the illites, the chlorites, the attapulgites and the mixed layer clays. Typical examples of specific clays belonging to these classes are:

smectites, e.g. montmorillonite, bentonite, pyrophyllite, hectorite, saponite, saucomite, nontronite, talc, beidellite, volchonskoite, vermiculite; kaolins, e.g. kaolinite, dickite, nacrite, antigorite, anauxite, halloysite, indellite, chrysotile; illites, e.g. bravaisite, muscovite, paragonite, phlogopite, biotite; chlorites, e.g. corrensite, penninite, donbassite, sudoite, pennine, clinochlore; attapulgites, e.g. sepiolite, polygorskite; mixed layer clays, e.g. allevardite, vermiculitebiotite.

The layered clay minerals may be either naturally occurring or synthetic. Preferred clay minerals for use in the present invention are natural or synthetic hectorites, montmorillonites and bentonites, and of these the hectorites are especially preferred. Many of the above clays are commercially available, and typical examples of commercial hectorites are the Laponites from Laporte Industries Ltd, England; Veegum Pro and Veegum F from R. T. Vanderbilt, U.S.A.; the Barasyms, Macaloids and Propaloids from Baroid Division, National Lead Comp., U.S.A.

A useful procedure for producing the present gelled organic liquids comprises dissolving the anionic polymer in the organic solvent. This is usually accomplished with

moderate mixing. The mixing is continued until there is a homogeneous solution. The auxiliary rheological additive, alone or as an aqueous or organic solution or dispersion, is then added to the solution of the anionic polymer. This is added with moderate mixing. An amphoteric oxide is added as a dispersion in water or an organic liquid. After the auxiliary rheological additive has been added and a homogeneous mixture formed, the amine is added to neutralize the polymer. During the initial addition, the homogenous mixture may thicken quickly and then become viscous. This can be expected. The amine is added while the homogenous mixture is being vigorously mixed. The resulting gelled organic liquid has very good thixotropic properties.

A primary advantage in using an auxiliary Theological additive is that less of the anionic polymer and amine neutralizing agent needs to be used to reach the same levels of viscosity. The amount of anionic polymer can be decreased by about 10 percent up to about 75 percent by weight, and preferably by at about 20 percent to 60 percent by weight and by at least about 25 percent by weight and replaced by the auxiliary rheological agent. At these decreased anionic polymer levels the viscosity remains at a high level if the auxiliary rheological additive is in an amount to compensate for the loss in viscosity due to the decrease in anionic polymer. The replacement with auxiliary Theological additive can be on a basis of about 0.01 to 5 parts of auxiliary rheological agent for each part of anionic polymer removed and usually about 0.5 to 2.5 parts.

If the amount of anionic polymer is not decreased the viscosity of the polymeric gel is increased 10 to 300 percent by weight and usually about 20 to 100 percent. This is an inexpensive way to increase the viscosity of polymeric gel.

When fuel compositions are gelled it is desirable to keep the anionic polymer and amine neutralizing agent to as low a level as possible. Although amounts of up to 10 percent by weight can be used, an increased level of anionic polymer and amine will result in a residue remaining after all of the fuel has been burned. Such a residue will smolder in the fuel container and emit smoke and odorous fumes at the end of a burn time. This is a distinct disadvantage when used to heat chafers at a banquet. The amount of anionic polymer must be kept below an amount that would leave a residue that would smolder after the fuel has been consumed. In this regard it is preferred that the anionic polymer be in a content of less than about 3 percent by weight, preferably less than about 1.5 percent and most preferably less than about 0.75 percent. A decreased amount of amine neutralizing agent is used to neutralize a decreased amount of anionic polymer.

It also is preferred in fuel compositions that the auxiliary rheological agent be an amphoteric oxide. Amphoteric oxides prevent the formation of a skin seal layer at the burn front with a resulting crackling noise and spouting as the vaporized fuel breaks through this skin seal layer. Although in fuel compositions the amphoteric oxide auxiliary rheological agent can be in a content of up to about 10 percent by weight, it will preferably be in a content of less than about 4 percent by weight, more preferably less than about 2 percent and most preferably less than about 0.75 percent. It is theorized that the amphoteric oxide provides pores at the burn front so that fuel can readily vaporize and burn. The key factor is that the amphoteric oxide should not be in a concentration wherein after the fuel has been consumed it would promote smoldering through the adsorption of the neutralized anionic polymer on the amphoteric oxide.

#### EXAMPLES 1-6

In this set of runs, Examples 1-3 are ethanol fuel gel compositions that contain a polyacrylic acid thickening

## 15

agent but no alumina auxiliary rheological additive, while examples 4–6 are ethanol fuel gel compositions that contain a polyacrylic acid thickening agent and an alumina auxiliary rheological additive. The polyacrylic polymer is B.F. Goodrich Carbopol 676 and the alumina is Dispal Alumina 23N4-80 available from the Vista Chemical Corporation.

The gelled ethanol compositions were prepared according to the following procedure. The Carbopol 676 polymer was slowly sieved (16 or 20 Mesh) and added into the ethanol with mixing at a temperature of about 25° C. and mixing was continued for fifteen minutes. A solution of the alumina was prepared by slowly adding with mixing the Dispal Alumina 23N4-80 and mixing was continued for about ten minutes. The diisopropanolamine was added with mixing at room temperature to the solution of water and Dispal Alumina 23N4-80 to water and mixing was continued for ten minutes. To the solution of the Carbopol 676 polymer and ethanol was quickly added with mixing the solution of the diisopropanolamine and Dispal Alumina 23N4-80 and mixing was continued for about two minutes.

The composition of the gelled ethanol are given in Table 2. The viscosity of the gelled ethanol in centipoise is given in Table 3. The viscosity is a Brooksfield viscosity at 10 rpm with a spindle #7 at room temperature. It is seen that the alumina containing compositions have a higher initial and long time viscosity than non-alumina containing compositions. In addition, over time the alumina containing compositions maintain a higher viscosity compared to the compositions that do not contain alumina.

In these Examples, Examples 1 and 4 are compared as are Examples 2 and 5 and Examples 3 and 6. By the addition of the alumina additive the viscosity in Example 4 is increased 53.5%. In Example 5 the viscosity increase is 50.0% over that of Example 2. And for Example 6 the viscosity increase is 56.9% over that of Example 3. These are significant increases in viscosity through the use of an auxiliary rheological additive.

TABLE 2

| COMPONENTS           | EXAMPLE |       |       |       |       |       |
|----------------------|---------|-------|-------|-------|-------|-------|
|                      | 1       | 2     | 3     | 4     | 5     | 6     |
| Polyacrylate Polymer | 0.75    | 0.65  | 0.55  | 0.75  | 0.65  | 0.55  |
| Ethanol              | 71      | 71    | 71    | 71    | 71    | 71    |
| Water                | 27.25   | 27.35 | 27.45 | 26.75 | 26.85 | 26.95 |
| Alumina              | 0       | 0     | 0     | 0.5   | 0.5   | 0.5   |
| Diisopropanolamine   | 1       | 1     | 1     | 1     | 1     | 1     |

TABLE 3

| DAYS    | EXAMPLE |        |        |         |         |         |
|---------|---------|--------|--------|---------|---------|---------|
|         | 1       | 2      | 3      | 4       | 5       | 6       |
| Initial | 86,000  | 76,000 | 68,000 | 116,800 | 103,600 | 89,200  |
| 1       | 86,400  | 76,000 | 71,200 | 131,600 | 116,400 | 92,000  |
| 2       | 87,200  | 81,200 | 63,200 | 136,400 | 120,000 | 102,800 |
| 7       | 86,400  | 84,000 | 76,400 | 130,000 | 126,000 | 113,600 |
| 14      | 90,000  | 90,400 | 78,000 | 134,000 | 127,200 | 116,000 |
| 28      | 93,200  | 89,200 | 82,000 | 132,000 | 126,400 | 110,400 |
| 42      | 94,000  | 96,000 | 84,000 | 130,000 | 132,400 | 110,400 |
| 56      | 81,600  | 93,600 | 78,000 | 128,400 | 125,600 | 126,000 |
| 84      | 104,000 | 89,200 | 81,600 | 159,600 | 132,000 | 128,000 |

## EXAMPLES 7–12

In this set of runs, Examples 7–9 are methanol fuel gel compositions that contain a polyacrylic acid thickening agent

## 16

but no alumina, while Examples 10–12 are methanol fuel gel compositions that contain a polyacrylic acid thickening agent and alumina. The polyacrylic polymer is B.F. Goodrich Carbopol 676 and the alumina is Dispal Alumina 23N4-80 available from Vista Chemical Corporation.

The gelled methanol compositions were prepared according to the following procedure. The Carbopol 676 polymer was slowly sieved (16 or 20 Mesh) and added into the methanol with mixing at a temperature of about 25° C. and mixing was continued for fifteen minutes.

A solution of the alumina was prepared by slowly adding with mixing the Dispal Alumina 23N4-80 and mixing was continued for about ten minutes. The diisopropanolamine was added with mixing at room temperature to the solution of water and Dispal Alumina 23N4-80 and mixing was continued for ten minutes. To the solution of the Carbopol 676 polymer and methanol was quickly added with mixing the solution of the diisopropanolamine and the Dispal Alumina 23N4-80 and mixing was continued for two minutes.

The composition of the gelled methanol are given in Table 4. The viscosity of the gelled methanol in centipoise is given in Table 5. The viscosity is a Brookfield viscosity at 10 rpm and a spindle #7 at room temperature. It is seen that the alumina containing compositions have a higher initial and long time viscosity than non-alumina containing compositions. In addition, over time the alumina containing compositions maintain a higher viscosity compared to the compositions that do not contain alumina.

In these Examples 7 to 12 the comparative examples are Examples 7 and 10, Examples 8 and 11 and Examples 9 and 12. Example 10 shows a 52.5% viscosity increase over that of Example 7. Example 11 shows a 76.0% increase over the viscosity of Example 8 and Example 12 shows a 31% increase in viscosity. The presence of the alumina auxiliary rheological additive shows a pronounced increased in the viscosity of the gels.

TABLE 4

| COMPONENTS           | EXAMPLE |       |       |       |       |       |
|----------------------|---------|-------|-------|-------|-------|-------|
|                      | 7       | 8     | 9     | 10    | 11    | 12    |
| Polyacrylate Polymer | 0.75    | 0.65  | 0.55  | 0.75  | 0.65  | 0.55  |
| Methanol             | 72      | 72    | 72    | 72    | 72    | 72    |
| Water                | 26.25   | 26.35 | 26.45 | 25.75 | 25.85 | 25.95 |
| Alumina              | 0       | 0     | 0     | 0.5   | 0.5   | 0.5   |
| Diisopropanolamine   | 1       | 1     | 1     | 1     | 1     | 1     |

TABLE 5

| DAYS    | EXAMPLE |        |        |         |         |         |
|---------|---------|--------|--------|---------|---------|---------|
|         | 7       | 8      | 9      | 10      | 11      | 12      |
| Initial | 82,400  | 73,200 | 60,000 | 100,400 | 97,600  | 66,000  |
| 1       | 94,000  | 79,200 | 58,000 | 118,800 | 114,400 | 84,800  |
| 2       | 87,200  | 84,000 | 64,800 | 132,000 | 127,600 | 106,000 |
| 7       | 98,400  | 79,200 | 71,200 | 136,000 | 117,600 | 80,000  |
| 14      | 91,600  | 91,600 | 76,400 | 124,000 | 112,000 | 112,000 |
| 28      | 84,400  | 80,000 | 70,400 | 144,000 | 132,000 | 116,800 |
| 42      | 92,400  | 86,800 | 81,600 | 156,800 | 137,600 | 92,000  |
| 56      | 94,400  | 77,200 | 79,600 | 144,000 | 134,800 | 109,200 |

## EXAMPLE 13

The composition of Example 6 was prepared and filled into formed aluminan containers having an internal diameter of 8.64 cm and a height of 6.35 cm. The top opening is 5.08 cm. The average weight of gelled ethanol fuel is 221.7 g.

## 17

One container is placed under a chafing dish containing 3 liters of water at 43° C. in the water pan portion of the chafing dish and 2 liters of water 43° C. in the food pan. This container is ignited and from thermocouples in the water pan and food pan the temperatures of water in these pans are recorded. The averaged data for the runs is as follows:

|                  |                |
|------------------|----------------|
| Burn Time        | 131 minutes    |
| Burn Rate        | 1.49 g/min     |
| Min To 65.5° C.  |                |
| Water Pan        | 24.25 minutes  |
| Min To 65.5° C.  |                |
| Food Pan         | 54 minutes     |
| Min To Max T° C. |                |
| Water Pan        | 122 minutes    |
| Min To Max T° C. |                |
| Food Pan         | 129.75 minutes |
| Max T° C.        |                |
| Water Pan        | 99.1° C.       |
| Max T° C.        |                |
| Food Pan         | 89.1° C.       |

This example shows the canned fuels to have an acceptable burn time and temperature profile. There was no sputtering or noise caused by a skin formation on the surface of the gel during burning.

## EXAMPLE 14

The fuels of Example 13 were tested for conformance with tested according to ASTM D 4359-84. The title of this test is "Determining Whether A Material Is A Liquid Or A Solid". The fuels are placed in quart cans and filled to at least the 85 percent (85%) level. The cans are sealed using friction lids and placed in an oven at 38° C.±3° C. for 24 hours. The cans are then removed from the oven and the lids removed. The cans are placed inverted in a stand for 3 minutes. The level of the gelled fuel in the can is measured at the start and end of the 3 minute period. A flow of 5 cm or less is acceptable and the material is considered to be a solid. The canned fuel samples that were tested. There was no flow. They are classified as solids under ASTM D 4359-84.

## EXAMPLES 15-36

The formulas (15-36) were prepared according to the following procedure. The Carbopol 676 polymer was slowly sieved (16 or 20 Mesh) and added into the methanol or ethanol with mixing at a temperature of about 25° C. and mixing was continued for fifteen minutes. A solution of the alumina was prepared by slowly adding with mixing the Dispal Alumina 23N4-80 and mixing was continued for about ten minutes. The diisopropanolamine was added with mixing at room temperature to the solution of water and Dispal 23N4-80 and mixing was continued for ten minutes. To the solution of the Carbopol 676 polymer and methanol (or ethanol) was quickly added with mixing the solution of the diisopropanolamine and the Dispal Alumina 23N4-80 and mixing was continued for two minutes. The Brookfield viscosities in centipoise were run at room temperature using a #7 spindle at 10 rpm.

These examples illustrate various properties. In Examples 15-17 it is shown that an increase in alkalinity has a deleterious effect on viscosity. In Examples 18-25 it is seen that in each instance where alumina is added to a given Carbopol 676 level that the viscosity is increased by about 20 to 40 percent. This is a significant increase in viscosity. Similar dramatic increases in viscosity are shown in Example 26-36. Here at different levels of Carbopol 676 there are comparisons of the alumina additive being present.

## 18

The viscosity of these alcohol gels can be significantly increased by the addition of relatively small amount of an inexpensive alumina additive.

## EXAMPLE 37

The Complex Viscosities (Pa.s), the Storage Moduli G' (N/m<sup>2</sup>), and the Loss Moduli G" (N/m<sup>2</sup>) of Compositions at 150 micro N.m and 10 rad/s (Strain Sweep Experiment) were obtained. Methanol (34)=0.45% Carbopol, Methanol (35)=0.45% Carbopol plus 0.5% Alumina, Ethanol (24)=0.45% Carbopol, and Ethanol (25)=0.45% Carbopol plus 0.5% Alumina.

|                               | Ethanol (24) | Ethanol (25) | Methanol (34) | Methanol (35) |
|-------------------------------|--------------|--------------|---------------|---------------|
| Complex Viscosity (Pa · s)    | 40.13        | 52           | 39.10         | 75.28         |
| G'(N/m <sup>2</sup> )         | 398.9        | 517.6        | 389.2         | 750.6         |
| G"(N/m <sup>2</sup> )         | 44.58        | 49.48        | 37.64         | 57.79         |
| Yield Stress N/m <sup>2</sup> | 85.53        | 124.6        | 87.37         | 91.08         |

Pa = NM<sup>-2</sup>  
N/m<sup>2</sup>  
39.10 Pa · s = 391.0 dyne · cm<sup>-2</sup> · s  
359.2 N/m<sup>2</sup> = 3892 dyne · cm<sup>-2</sup>

## EXAMPLE 38

30 A series of gelled ethanol fuels were prepared by forming a mixture of ethanol, Carbopol 676, blue dye, Bitrex and fragrance as a first component. A second component consisting of water, Dispal Alumina 23N4-20 sol and diisopropanolamine was added to the first component. The mixture contains 76.45 percent ethanol, 0.55 percent Carbopol 676, 19.9 percent water, 0.40 percent Dispal Alumina 23N4 and 0.85 percent diisopropanolamine. After mixing and the formation of the gel the nominal viscosity after 24 hours is 85,000 to 100,000 centipoise.

35 Eight ounces of the formulation when placed in a container having an internal diameter of 84 mm, a height of 62 mm, and a burner opening of 49.7 mm burns nominally for 130 minutes. The composition burns silently with no sputtering or crackling which would be evidence of film formation at the burn front. The composition also can be easily relit if extinguished. This is a function of the alumina additive.

## EXAMPLE 39

50 A series of gelled methanol fuels were prepared by forming a mixture of methanol, Carbopol 676, blue dye, Bitrex and fragrance as a first component. A second component consisting of water, Dispal Alumina 23N4-20 sol and diisopropanolamine was added to the first component. The mixture contains 71 percent methanol, 0.5 percent Carbopol 676, 25.5 percent water, 0.40 percent Dispal Alumina 23N4 and 0.85 percent diisopropanolamine. After mixing and the formation of the gel the viscosity after 24 hours is 80,000 to 95,000 centipoise.

55 Seven ounces of the formulation when placed in a container having an internal diameter of 84 mm, a height of 62 mm and a burner opening of 49.7 mm burns nominally for 130 minutes. The composition burns silently with no sputtering or crackling which would be evidence of film formation at the burn front. The composition also can be easily relit if extinguished. The presence of the alumina additionally functions to permit the easy relighting of the fuel.

## 19

What is claimed is:

1. A polymeric gel having increased viscosity provided by an auxiliary rheological additive comprising approximately by weight:

- (a) 0.1 to 10.0 weight percent of an anionic polymer at least partially neutralized through the addition of at least one organic base to neutralize said anionic polymer and to form a gel; and
- (b) 0.01 to 10.0 percent by weight of an amphoteric oxide auxiliary rheological additive; and
- (c) the balance being primarily at least one organic solvent;

wherein the polymeric gel is viscoelastic and has a  $G'$  value of at least 80 dynes/sq. cm at a frequency of 10 radians/second, a  $G''$  value of at least 10 dynes/sq. cm. at a frequency of 10 radians/second, a ratio of  $G''/G'$  of less than 1,  $G'$  being substantially constant over a torque range of 1 to 100 micro N.m. with the viscosity of the polymeric gel being increased by such auxiliary rheological additive such that the content of the anionic polymer in the polymeric gel can be decreased by 10 percent to 75 percent by weight and replaced with said auxiliary rheological additive and the polymeric gel has essentially an equivalent viscosity due to the presence of said auxiliary rheological additive.

2. A polymeric gel as in claim 1 wherein said at least one organic base is an amine.

3. A polymeric gel as in claim 2 wherein said anionic polymer is a cross-linked polyacrylic acid.

4. A polymeric gel as in claim 3 wherein said auxiliary rheological additive is alumina.

5. A polymeric gel as in claim 1 wherein the auxiliary rheological additive is an alumina.

6. A polymeric gel as in claim 1 wherein said solvent is a fuel.

7. A polymeric gel as in claim 6 wherein said fuel is selected from the group consisting of alkanes, alkenes, alcohols of from 1 to 6 carbon atoms, aromatic hydrocarbons and mixtures thereof.

8. A polymeric gel as in claim 7 wherein said alcohol is selected from the group consisting of methanol, ethanol and mixtures thereof.

9. A polymer gel as in claim 1 wherein said polymeric gel is viscoelastic and is solid under ASTM D 4359-84.

10. A polymer gel as our claim 1 wherein the polymeric gel has a  $G'$  value of at least 2500 dynes/sq. cm at a frequency of 10 radians/second, a  $G''$  value of at least 200 dynes/sq. cm. at a frequency of 10 radians/second, a  $G''/G'$  ratio of less than 1, and  $G'$  being substantially constant over a torque range of 1 to 150 micro N.m.

## 20

11. A polymeric gelled fuel composition having an increased viscosity provided by an auxiliary rheological additive comprising approximately by weight:

- (a) 0.1 to 3 percent by weight of an anionic polymer at least partially neutralized through the addition of at least one organic base to neutralize said anionic polymer and to form a gel;
- (b) 0.01 to 4 percent by weight of an amphoteric oxide auxiliary rheological additive; and
- (c) the balance being primarily a fuel;

wherein the polymeric gel is viscoelastic and has a  $G'$  value of at least 80 dynes/sq. cm at a frequency of 10 radians/second, a  $G''$  value of at least 10 dynes/sq. cm. at a frequency of 10 radians/second, a ratio of  $G''/G'$  of less than 1,  $G'$  being substantially constant over a torque range of 1 to 100 micro N.m. with the viscosity of the polymeric gel being increased by said auxiliary rheological additive such that the content of the anionic polymer in the polymeric gel can be decreased by 10 percent to 75 percent by weight and the polymeric gel has essentially an equivalent viscosity due to the presence of said auxiliary rheological additive.

12. A polymeric gelled fuel composition as in claim 11 wherein said fuel is selected from the group consisting of alkanes, alkenes, alcohols of from 1 to 6 carbon atoms, aromatic hydrocarbons and mixtures thereof.

13. A polymeric gelled fuel composition as in claim 12 wherein said fuel is selected from the group consisting of methanol, ethanol and mixtures thereof.

14. A polymeric gelled fuel composition as in claim 13 wherein said fuel is methanol.

15. A polymeric gelled fuel composition as in claim 13 wherein said fuel is ethanol.

16. A polymeric gelled fuel composition as in claim 12 wherein said anionic polymer is in an amount of less than about 1.5 percent and said amphoteric oxide is in an amount of less than about 2 percent.

17. A polymeric gelled fuel composition as in claim 16 wherein said anionic polymer is in an amount of less than about 0.75 percent and said amphoteric is in an amount of less than about 0.75 percent.

18. A gelled fuel composition as in claim 17 wherein said gelled fuel composition is viscoelastic and is solid under ASTM D 4359-84.

19. A gelled fuel composition as in claim 17 wherein the polymeric gel has a  $G'$  value of at least 2500 dynes/sq. cm at a frequency of 10 radians/second, a  $G''$ .

\* \* \* \* \*

UNITED STATES PATENT AND TRADEMARK OFFICE  
**CERTIFICATE OF CORRECTION**

PATENT NO. : 5,773,706

DATED : June 30, 1998

INVENTOR(S) : John N. Wesley, Amjad Farooq, Ammanuel Mehreteab,  
Francis T. Barbato

It is certified that error appears in the above-identified patent and that said Letters Patent is hereby corrected as shown below:

In Column 20, Claim 19, please add the following language before the period to complete Claim 19:

"value of at least 200 dynes/sq. cm. at a frequency of 10 radians/second, a G"/G' ratio of less than 1, and G' being substantially constant over a torque range of 1 to 150 micro N.m."

Signed and Sealed this  
Eleventh Day of May, 1999

Attest:



Q. TODD DICKINSON

Attesting Officer

Acting Commissioner of Patents and Trademarks